

June 4, 1935.

A. N. GRAY

2,003,772

INSULATED CONDUCTOR

Filed Dec. 16, 1930



INVENTOR  
A. N. GRAY  
BY  
H. J. Banfield  
ATTORNEY

## UNITED STATES PATENT OFFICE

2,003,772

## INSULATED CONDUCTOR

Alvin N. Gray, Baltimore, Md., assignor to Bell Telephone Laboratories, Incorporated, New York, N. Y., a corporation of New York

Application December 16, 1930, Serial No. 502,667

9 Claims. (Cl. 173—264)

This invention relates to insulated conductors and more particularly to insulated conductors wherein the conducting element comprises very fine conducting wires or strips.

5 In certain branches of the telephone industry it is desirable to employ flexible conductors, for example, the well known tinsel cord conductors used in connection with telephone handsets must be extremely flexible to permit frequent bending 10 and twisting without impairing the transmission characteristics of the set. To obtain this flexibility such conductors are made up of a number of very fine conducting wires or strips suitably grouped together. Furthermore, when such conductors are to be employed in damp places it is the usual practice to protect such conductors 15 against corrosion by applying a protective coating of vulcanized rubber insulation. In applying this layer of rubber it is the present practice 20 to bring about vulcanization with the aid of sulphur and an accelerating agent. In the case of ordinary conductors wherein the cross-section of the conducting wires or strips that go to make up the conductor is relatively large this process 25 is fairly satisfactory. However, in cases where this cross-section of the conducting wires or strips is relatively small, for example, in the case of tinsel cord conductors, this process is 30 very unsatisfactory since in such cases the free sulphur which is ordinarily liberated in time corrodes the conducting wires or strips to a point where they are unsatisfactory for service or even where they are completely destroyed thus defeating 35 the purpose for which the layer of rubber insulation was primarily applied.

The object, therefore, of the present invention is to produce an insulated conductor comprising one or more fine conducting wires or strips, the transmission characteristics of which are 40 main substantially constant.

In accordance with the present invention this object is attained by coating the conductor with a layer of rubber composition and then vulcanizing this composition with the aid of such 45 agents that the amount of sulphur which remains uncombined is reduced to a minimum. In accordance with the preferred process the rubber composition is vulcanized with the aid of sulphur and an organic accelerator such as tetra- 50 ramethylthiuramdisulfide or as it is generally called "Tuads". This "Tuads" however contains a certain percentage of sulphur which is liberated during the vulcanizing process and it has been found that the sulphur thus liberated when 55 combined with the sulphur ordinarily added produces an excess of sulphur which remains uncombined and is available therefore as a corrosive agent. By properly proportioning the amount of sulphur which is ordinarily added 60 and the amount of sulphur in the accelerating

agent it is possible to make available just the amount of sulphur needed to produce a satisfactory vulcanization without leaving uncombined sulphur in the composition.

In accordance with a modification of this process the rubber composition is vulcanized with the aid of "Tuads" alone. In this modification a sufficient amount of "Tuads" is added to the mixture so that the sulphur which is liberated is sufficient to produce satisfactory vulcanization without leaving uncombined sulphur in the composition. 5

The use of such compounds, that is sulphur and "Tuads", is old in the art of vulcanizing rubber having been used heretofore to increase 15 the speed of vulcanization but as far as applicant is aware no one prior to applicant's invention has conceived the idea of properly proportioning the amount of the vulcanizing agents to prevent corrosion on fine conducting wires 20 caused by a certain percentage of the added sulphur remaining uncombined in the rubber compound.

A clearer understanding of this invention may be had by reference to the accompanying 25 drawing which shows a conductor insulated in accordance with the present invention.

As shown by the drawing a tinsel cord conductor is made up of a number of individual conductors, each individual conductor comprising 30 a very fine conducting wire or strip 10 helically wrapped around a strand of textile material 11. The conductors thus formed are then preferably twisted about a core of textile material 13 to obtain the necessary mechanical 35 strength and are then bound together by two servings 14 and 15 of textile material which are wound about the conductor in opposite directions. When these conductors are to be employed in damp places they are protected against 40 corrosion by applying a protective coating of vulcanized rubber insulation 16. Two such conductors are usually grouped together and held in place by an outer braiding of textile material 17. In accordance with the present practice 45 the layer of rubber is applied by extruding a mass of rubber containing sulphur and an accelerating agent about the conductor and then applying heat. During the heating the sulphur, under the influence of the accelerating agent, 50 combines with the rubber and thus brings about vulcanization. During this process however it has been found that a certain amount of the sulphur remains free or uncombined and is therefore present as a corrosive agent. In the 55 case of the ordinary conductor the corrosive action produced by the uncombined sulphur is relatively unimportant but it becomes of vital importance in the case of the tinsel cord conductors wherein the thickness of individual con- 60

ducting strips is in the neighborhood of approximately 1 mil since in such cases the corrosion soon renders the conductors unsatisfactory and in some cases may completely destroy the conductor thus defeating the purpose for which the layer of rubber insulation was primarily employed.

In accordance with the preferred form of the present invention this corrosive action is avoided by vulcanizing the layer of rubber composition with the aid of sulphur and an organic accelerator such as tetramethylthiuramdisulfide or, as it is generally called "Tuads", the percentages of the sulphur and "Tuads" used being such that no uncombined sulphur remains in the compound after vulcanization. While the following formula is preferred yet it is to be understood that it is given merely for the purpose of illustration and that the various elements and the percentages thereof may be varied as occasion demands:

|                             |      |
|-----------------------------|------|
| Pale crepe rubber           | 32.0 |
| Reclaimed white rubber      | 20.0 |
| Tetramethylthiuramdisulfide | 1.0  |
| 25 Sulphur                  | 0.3  |
| Zinc oxide                  | 3.0  |
| Neozone                     | 1.0  |
| Stearic acid                | 0.2  |
| Di-phenyl-guanidine         | 0.5  |
| 30 Whiting                  | 42.0 |

After the above composition has been thoroughly mixed a coating of a predetermined thickness is extruded about a conductor in any suitable manner. The conductor thus coated is then covered with talc and placed in a vulcanizer where it is heated for approximately 20 minutes to about 275° F. During this heating process the sulphur combines with the rubber and brings about vulcanization, the rate of vulcanization depending to a great extent upon the amount of accelerator used. Inasmuch as the "Tuads" contains a certain percentage of sulphur which is freed during the heating, it is necessary to carefully proportion the amount of sulphur and the amount of "Tuads", otherwise there will be a certain percentage of sulphur which will remain uncombined and thus corrode the very fine conducting strips.

While the foregoing is the preferred method of vulcanizing the rubber composition yet good results may be obtained by the use of "Tuads" alone. In this case the percentage of the "Tuads" is increased to the point where the sulphur which is freed during the heating of the "Tuads" is just sufficient to produce a thorough vulcanization without leaving any uncombined sulphur.

What is claimed is:

1. The method of preventing corrosion of conductors which consists in coating said conductors with a rubber compound and vulcanizing said compound with the aid of sulphur and an organic accelerator containing sulphur, said organic accelerator being added in sufficient quantities to bring the sulphur content of the mixture to the predetermined value required to cause the vulcanizing action to go to completion with the elimination of free sulphur in the resulting vulcanized rubber.

2. The method of preventing corrosion of conductors which consists in coating said conductors with a rubber compound and vulcanizing

said compound with the aid of sulphur and tetramethylthiuramdisulfide which are added to the rubber compound in such quantities as to bring the total sulphur content to the predetermined value necessary to carry the vulcanization reaction to completion without leaving any uncombined sulphur in the vulcanized product.

3. The method of preventing corrosion of conductors which consists in coating said conductors with a rubber compound containing a known percentage of sulphur and vulcanizing said compound with the aid of tetramethylthiuramdisulfide which is limited in amount so that the sulphur released from it during the vulcanization process together with that contained in said rubber compound will be just sufficient to carry the reaction to completion without leaving uncombined sulphur in the resulting insulating layer.

4. The method of insulating an electrical conductor which comprises extruding a rubber composition containing at least one per cent of tetramethylthiuramdisulfide and substantially three tenths of one per cent sulphur and vulcanizing said composition under the influence of heat.

5. The method of preventing corrosion of conductors which consists in coating said conductors with a rubber composition containing a known percentage of sulphur, vulcanizing said composition with the aid of sulphur containing accelerating agents such as tetramethylthiuramdisulfide and a non-sulphur containing accelerating agent such as diphenylguanidine, said tetramethylthiuramdisulfide being quantitatively added to increase the sulphur content of the mixture to an amount required to cause the reaction to go only to completion, without leaving any uncombined sulphur in the vulcanized product.

6. The method of preventing corrosion of conductors which consists in coating said conductors with a rubber composition containing a known percentage of sulphur, vulcanizing said composition with the aid of a tetraalkylated thiuramdisulfide and a disubstituted guanidine, said thiuramdisulfide being added to increase the sulphur content of the mixture to an amount required to cause the reaction to go only to completion without leaving any uncombined sulphur in the vulcanized product.

7. An electrical conductor comprising a conducting core and a layer of vulcanized insulation thereupon containing before vulcanization approximately 1 part of tetramethylthiuramdisulfide and 0.3 parts of sulphur to 39 parts of rubber.

8. An electrical conductor comprising a conducting core and a layer of vulcanized insulation thereupon, free from uncombined sulphur, said insulation containing before vulcanization free sulphur, a sulphur containing accelerator and a non-sulphur containing accelerator.

9. An electrical conductor, comprising a conducting core and a layer of vulcanized rubber compound thereon, which rubber compound contained before vulcanization free sulphur and a sulphur containing organic accelerator in such proportions that upon vulcanization the compound is completely vulcanized but substantially no free sulphur remains therein.

ALVIN N. GRAY.